

Patented Sept. 19, 1922.

1,429,467

# UNITED STATES PATENT OFFICE.

PEARL E. ULLRICH, OF CHICAGO, ILLINOIS.

## BELT DRESSING.

No Drawing.

Application filed October 30, 1920. Serial No. 420,793.

To all whom it may concern:

Be it known that I, PEARL E. ULLRICH, a citizen of the United States, residing at Chicago, in the county of Cook and State of Illinois, have invented a certain new and useful Improvement in Belt Dressings, of which the following is a full, clear, concise, and exact description.

My invention relates to belt dressings.

10 In providing a suitable compound for conditioning and preserving leather driving belts, it is essential to provide a constituent which will keep the belt soft and pliable and preserve the same against deterioration, 15 and at the same time to provide a surfacing compound which will increase the grip or friction between the pulley and the belt.

I have discovered that base oil in condensed form is suitable for use as a belt 20 dressing, as it contains the necessary properties for preserving the leather of the belt, and also providing a satisfactory surfacing to maintain the grip of the belt upon the pulley.

25 In the manufacture of water gas an incandescent body of coal is treated with steam to form what is known as dry gas. The gas is then enriched or carburetted by cracking a petroleum oil known as gas oil, 30 which is a petroleum distillate of a boiling point of from about 500° F. to 700° F.

About 65% of this oil by weight is transformed into a fixed gas, and about 20% forms a residue of an oil tar, some carbon being 35 formed.

The gas is then cooled and scrubbed, and at this stage certain grades of oil known as wash oils are extracted from the gas.

40 The heavier of these wash oils are extracted first. Thereafter, what is known as light oils are extracted. The heavier and lighter grades may all be run off together.

About 10% of the wash oils have boiling points at or below 200° C., beginning with 45 benzine at about 81° C., toluene at about 110° C., xylenes at about 140° C., cymenes at about 170° C., and still others at higher points and with numerous grades between these points. The xylenes and cymenes are 50 known as solvent oils.

My invention employs the residue of the light oils after the aromatic oils, or solvents, have been fractioned off. This residue is known as base oil and forms the source 55 of material for my improved belt dressing.

The base oil as it comes from the still or

by-product plant is a thin, brown, oily liquid having a strong gas odor. This oil when rubbed between the fingers finally leaves a thin coating, somewhat greasy, but apparently of little lubricating character.

This raw base oil is too thin to be suitable for my purpose, and I therefore thicken or condense the same by heating over an open flame in the presence of air. In the manufacture which I have thus far conducted, I have heated the base oil at this stage to the boiling point in the presence of the oxygen of the atmosphere, and I have agitated the mass by stirring. I consider that the agitation could be accompanied by blowing of air through the base oil. I consider that the heating has resulted, first of all, in driving off some of the lighter oils, and second perhaps in polymerization of some of the mass 75 to thicken the same, and third, the oxygen of the air appears to promote the viscosity of the oil.

I propose to manufacture the composition on a larger scale than at present by heating 80 the oil with steam coils and blowing air and steam therethrough, both to secure agitation and to bring the oxygen of the air in contact with the hot base oil.

The resultant material is a thick liquid 85 mass of specific gravity substantially 1.018 at 15½° C., and a viscosity of substantially 10.9 at a temperature of 140° C., as compared with water at 20° C., as measured by the Saybolet viscosometer.

I consider that the mass contains a certain amount of oil, with other constituents, the nature of which I am unable to explain, and which I beg leave to describe more in detail as soon as I become aware of the true 95 character thereof. The thinner oils serve to keep the belt flexible and well preserved, and the other constituents serve to impart a surfacing which grips the pulley. The belt dressing of my invention is of a substantially 100 fixed character, as it does not deteriorate with age, nor does it tend to evaporate when exposed to the atmosphere. It is free from any injurious constituents which would attack the leather of the belt, and at the same 105 time it provides an adhesive surface which is capable of imparting the necessary gripping qualities to the leather.

After thickening or condensing the base oil in the manner above indicated, I prefer- 110 ably provide a masking odorant for over- coming the smell of gas which is given off by

this material. For this purpose oil of citronella, oil of sassafras or any suitable odorant of a relatively powerful character may be applied. This odorant has no effect so far as the conditioning and preserving of the belt is concerned; it is merely to make the product more salable.

The resulting material is packed in tins or the like and is applied to the belt in the well known manner.

I do not intend to be limited to the precise steps of procedure or the precise characteristics above described.

I claim:

- 15 1. A belt dressing consisting of concentrated base oil.
2. A belt dressing consisting of base oil of a specific gravity of substantially 1.018 at  $15\frac{1}{2}^{\circ}$  C.
- 20 3. A belt dressing consisting of the residue of wash oil from gas plants, after the

aromatic, or solvent hydrocarbons have been distilled.

4. The method of treating base oil to render the same suitable for belt dressing, which consists in heating the base oil to the boiling point until it assumes a specific gravity of substantially 1.018 at  $15\frac{1}{2}^{\circ}$  C.

5. A belt dressing consisting of condensed base oil of a viscosity of substantially 10.9 at a temperature of  $140^{\circ}$  C., as compared with water at  $20^{\circ}$  C.

6. A belt dressing consisting of a concentrated and aerated residue of wash oils from gas plants.

7. A belt dressing consisting of concentrated and oxidized residue of wash oils from gas plants.

In witness whereof, I hereunto subscribe my name this 28th day of October, 1920.

PEARL E. ULLRICH.